

## [54] INFECTIOUS DEVELOPER COMPOSITION

[75] Inventors: Isao Shimamura; Eiichi Okusut; Yoo Iijima; Haruhiko Iwano, all of Minami Ashigara-machi, Japan

[73] Assignee: Fuji Photo Film Co., Ltd., Ashigara-shi, Kanagawa, Japan

[22] Filed: Dec. 21, 1971

[21] Appl. No.: 210,546

## [30] Foreign Application Priority Data

Dec. 21, 1970 Japan..... 45-115432

[52] U.S. Cl. .... 96/66.4, 96/66 R

[51] Int. Cl. .... G03c 5/30

[58] Field of Search..... 96/66, 66.4

## [56] References Cited

## UNITED STATES PATENTS

|           |         |                 |       |         |
|-----------|---------|-----------------|-------|---------|
| 3,108,001 | 10/1963 | Green           | ..... | 96/66 R |
| 3,128,180 | 4/1964  | Henn            | ..... | 96/66.4 |
| 3,134,673 | 5/1964  | Ganguin         | ..... | 96/66 R |
| 3,186,843 | 6/1965  | Haas            | ..... | 96/66 R |
| 3,241,964 | 3/1966  | Land            | ..... | 96/66 R |
| 3,257,207 | 6/1966  | Green           | ..... | 96/66 R |
| 3,276,873 | 10/1966 | Green           | ..... | 96/66 R |
| 3,300,305 | 1/1967  | Pesch et al.    | ..... | 96/66 R |
| 3,490,905 | 1/1970  | Blake           | ..... | 96/66 R |
| 3,576,634 | 4/1971  | Woodward et al. | ..... | 96/66 R |
| 3,600,176 | 8/1971  | Haist et al.    | ..... | 96/66 R |

3,632,341 1/1972 Zacchia ..... 96/66.4

Primary Examiner—Norman G. Torchin

Assistant Examiner—M. F. Kelley

Attorney, Agent, or Firm—Richard C. Sughrue et al.

## [57] ABSTRACT

An infectious developer for photographic plates for printing containing at least one phenol compound represented by the following formula:



wherein R<sub>1</sub>, R<sub>2</sub>, R<sub>3</sub>, R<sub>4</sub> and R<sub>5</sub> which need not be identical are a hydrogen atom, a hydrocarbon group, a substituted hydrocarbon group, an alkoxy group, COOM, SO<sub>3</sub>M where M is a hydrogen atom, a water soluble cation or a hydrocarbon group, a halogen atom, S - R<sub>6</sub> where R<sub>6</sub> is a hydrocarbon group or a substituted hydrocarbon group, COR, where R<sub>7</sub> is a hydrogen atom, a hydrocarbon group or a substituted hydrocarbon group, or NR<sub>8</sub>R<sub>9</sub> where R<sub>8</sub> and R<sub>9</sub> are a hydrogen atom, a hydrocarbon group or a substituted hydrocarbon group.

9 Claims, No Drawings

## INFECTIOUS DEVELOPER COMPOSITION

## BACKGROUND OF THE INVENTION

## 1. Field of the Invention:

The present invention relates to an infectious developer used for making photographic printing plates, particularly an infectious developer having excellent preservability which is used for making photographic plates having good image quality.

## 2. Description of the Prior Art:

Photographic plate for printing can generally be produced by an infectious development of a lithotype photographic sensitive element typically used for producing a dotted or line drawing or a hard photographic sensitive element having high contrast and forming images of excellent sharpness. Known litho-type sensitive elements include lithofilm or lithoplate which is used for recording images on a printed original having a continuous gradation density by dividing the images into meshed dots so that a variation in density changes into a variation in the area of the dots, and litholine film or litholine plate which is used for a printed original having line drawings.

In order to divide the image into the meshed dots, a cross line glass screen or a contact screen is used. A half-tone plate is obtained by printing the image of the original onto the litho-type sensitive element through a screen and conducting development.

An ideal half-tone plate consists of dotted spots having a maximum density and a background having a minimum density. However, since any hard photographic sensitive element has an intermediate density, areas of intermediate density, called fringe areas, are always formed around the dots. Fringe is not desirable for plate making because it notably deteriorates the quality of printed images. The line drawing image is thought of as continuous series of dotted images. Accordingly, in litholine film or plate, areas of intermediate density are not desirable.

The developer used for producing photographic plates for printing using a lithotype sensitive element or another hard sensitive element is usually an alkaline infectious developer which contains a dihydroxybenzene type developing agent and an aldehyde-alkali hydrogen sulfite addition product as the preservative. Infectious developers of this kind have poor preservability as compared to common black-white developers because the amount of a free sulfite ion is small. In a developer having a low free sulfite ion concentration, the life of activated hydroquinone is kept for a long period of time and the hydroquinone is infectively activated and accumulated thereby. Consequently, images having a high contrast and low fringe are obtained since the development is carried out rapidly.

However, in developers having a high free sulfite ion concentration, the life of the activated hydroquinone is

short and the hydroquinone is not accumulated. Consequently, images having a low contrast and high fringe are obtained since the development is not carried out rapidly. There is thus an interaction between the free sulfite ion concentration and the quality of the images obtained on the photographic plate for printing.

Since it is essential for an infectious developer to have a good preservability, it is necessary to improve the preservability by adding an antioxidant other than the sulfite. For instance, it is known to add ascorbic acid to an infectious developer (Jap. Pat. Pub. Sho 44-28673). However, ascorbic acid has a poor stability because it is easily decomposed and it is particularly unstable when metal ions, such as copper or iron ions exist in the developer. Consequently the preservability of the developer is poor. Moreover, ascorbic acid has the fault that it somewhat hinders the progress of the development and causes deterioration of the quality of half-tone dots if added in large amounts.

20 The present inventors have found a fact that the preservability of an infectious developer is remarkably improved without bad influence upon image quality by adding at least one phenol compound represented by the following formula to the infectious developer:



wherein R<sub>1</sub>, R<sub>2</sub>, R<sub>3</sub>, R<sub>4</sub> and R<sub>5</sub> can be identical or different and can represent a hydrogen atom, hydrocarbon group, substituted hydrocarbon group, alkoxy group, COOM, SO<sub>3</sub>M (M represents a hydrogen atom, a water soluble cation or a hydrocarbon group), halogen atom, S - R<sub>6</sub> (R<sub>6</sub> represents a hydrocarbon group or substituted hydrocarbon group), COR<sub>7</sub> (R<sub>7</sub> represents a hydrogen atom, hydrocarbon group or substituted hydrocarbon group) or NR<sub>8</sub>R<sub>9</sub> (R<sub>8</sub> and R<sub>9</sub> represent each a hydrogen atom, hydrocarbon group or substituted hydrocarbon group).

## SUMMARY OF THE INVENTION:

The object of the present invention is to provide a developer especially for photographic plate for printing, which does not have a bad influence upon the quality of the formed images and has excellent preservability.

## DETAILED DESCRIPTION OF THE INVENTION:

In the following, typical examples of the compounds used in the present invention are shown. However, the scope of the present invention is not limited to these compounds.

| Compound number | R <sub>1</sub>  | R <sub>2</sub>  | R <sub>3</sub>  | R <sub>4</sub>  | R <sub>5</sub>  |
|-----------------|-----------------|-----------------|-----------------|-----------------|-----------------|
| 1.              | CH <sub>3</sub> | H               | H               | H               | H               |
| 2.              | H               | H               | H               | CH <sub>3</sub> | H               |
| 3.              | H               | H               | H               | H               | H               |
| 4.              | CH <sub>3</sub> | CH <sub>3</sub> | H               | H               | H               |
| 5.              | CH <sub>3</sub> | H               | H               | H               | H               |
| 6.              | CH <sub>3</sub> | H               | H               | CH <sub>3</sub> | H               |
| 7.              | CH <sub>3</sub> | H               | H               | H               | CH <sub>3</sub> |
| 8.              | H               | H               | CH <sub>3</sub> | CH <sub>3</sub> | H               |
| 9.              | H               | H               | CH <sub>3</sub> | CH <sub>3</sub> | CH <sub>3</sub> |
| 10.             | CH <sub>3</sub> | CH <sub>3</sub> | CH <sub>3</sub> | H               | H               |
| 11.             | CH <sub>3</sub> | H               | CH <sub>3</sub> | H               | CH <sub>3</sub> |
| 12.             | CH <sub>3</sub> | H               | CH <sub>3</sub> | H               | CH <sub>3</sub> |
| 13.             | H               | H               | CH <sub>3</sub> | CH <sub>3</sub> | CH <sub>3</sub> |

| Compound number | R <sub>1</sub>                     | R <sub>2</sub>                    | R <sub>3</sub>                                                                                          | R <sub>4</sub>                                       | R <sub>5</sub>                      |
|-----------------|------------------------------------|-----------------------------------|---------------------------------------------------------------------------------------------------------|------------------------------------------------------|-------------------------------------|
| 14.             | CH <sub>3</sub>                    | II                                | CH <sub>3</sub>                                                                                         | CH <sub>3</sub>                                      | H.                                  |
| 15.             | CH <sub>3</sub>                    | CH <sub>3</sub>                   | CH <sub>3</sub>                                                                                         | CH <sub>3</sub>                                      | H.                                  |
| 16.             | CH <sub>3</sub>                    | CH <sub>3</sub>                   | CH <sub>3</sub>                                                                                         | CH <sub>3</sub>                                      | H.                                  |
| 17.             | CH <sub>3</sub>                    | II                                | CH <sub>3</sub>                                                                                         | CH <sub>3</sub>                                      | CH <sub>3</sub>                     |
| 18.             | CH <sub>3</sub>                    | CH <sub>3</sub>                   | CH <sub>3</sub>                                                                                         | CH <sub>3</sub>                                      | CH <sub>3</sub>                     |
| 19.             | CH <sub>3</sub>                    | CH <sub>3</sub>                   | II                                                                                                      | CH <sub>3</sub>                                      | CH <sub>3</sub>                     |
| 20.             | C <sub>2</sub> H <sub>5</sub>      | H                                 | —CH <sub>3</sub>                                                                                        | CH <sub>3</sub>                                      | CH <sub>3</sub>                     |
| 21.             | H                                  | II                                | II                                                                                                      | II                                                   | H.                                  |
| 22.             | H                                  | II                                | II                                                                                                      | C <sub>2</sub> H <sub>5</sub>                        | H.                                  |
| 23.             | n-C <sub>3</sub> H <sub>7</sub>    | H                                 | H                                                                                                       | H                                                    | H.                                  |
| 24.             | H                                  | H                                 | H                                                                                                       | H                                                    | H.                                  |
| 25.             | H                                  | H                                 | H                                                                                                       | n-C <sub>3</sub> H <sub>7</sub>                      | H.                                  |
| 26.             | H                                  | n-C <sub>3</sub> H <sub>7</sub>   | H                                                                                                       | H                                                    | H.                                  |
| 27.             | H                                  | H                                 | H                                                                                                       | H                                                    | H.                                  |
| 28.             | H                                  | H                                 | H                                                                                                       | Iso-C <sub>3</sub> H <sub>7</sub>                    | H.                                  |
| 29.             | H                                  | H                                 | Iso-C <sub>3</sub> H <sub>7</sub>                                                                       | H                                                    | H.                                  |
| 30.             | CH <sub>3</sub>                    | H                                 | H                                                                                                       | CH <sub>3</sub>                                      | H.                                  |
| 31.             | Iso-C <sub>3</sub> H <sub>7</sub>  | CH <sub>3</sub>                   | H                                                                                                       | H                                                    | Iso-C <sub>3</sub> H <sub>7</sub> . |
| 32.             | Iso-C <sub>3</sub> H <sub>7</sub>  | CH <sub>3</sub>                   | CH <sub>3</sub>                                                                                         | H                                                    | H.                                  |
| 33.             | Iso-C <sub>3</sub> H <sub>7</sub>  | Iso-C <sub>3</sub> H <sub>7</sub> | C <sub>2</sub> H <sub>5</sub>                                                                           | H                                                    | H.                                  |
| 34.             | n-C <sub>4</sub> H <sub>9</sub>    | H                                 | Iso-C <sub>3</sub> H <sub>7</sub>                                                                       | H                                                    | H.                                  |
| 35.             | H                                  | H                                 | H                                                                                                       | H                                                    | H.                                  |
| 36.             | H                                  | H                                 | n-C <sub>4</sub> H <sub>9</sub>                                                                         | H                                                    | H.                                  |
| 37.             | Sec-C <sub>4</sub> H <sub>9</sub>  | H                                 | Sec-C <sub>4</sub> H <sub>9</sub>                                                                       | H                                                    | H.                                  |
| 38.             | t-C <sub>4</sub> H <sub>9</sub>    | H                                 | H                                                                                                       | H                                                    | H.                                  |
| 39.             | H                                  | H                                 | H                                                                                                       | t-C <sub>4</sub> H <sub>9</sub>                      | H.                                  |
| 40.             | H                                  | H                                 | t-C <sub>4</sub> H <sub>9</sub>                                                                         | H                                                    | H.                                  |
| 41.             | t-C <sub>4</sub> H <sub>9</sub>    | CH <sub>3</sub>                   | H                                                                                                       | H                                                    | H.                                  |
| 42.             | n-C <sub>4</sub> H <sub>9</sub>    | CH <sub>3</sub>                   | H                                                                                                       | H                                                    | H.                                  |
| 43.             | Sec-C <sub>4</sub> H <sub>9</sub>  | CH <sub>3</sub>                   | H                                                                                                       | H                                                    | H.                                  |
| 44.             | t-C <sub>4</sub> H <sub>9</sub>    | CH <sub>3</sub>                   | CH <sub>3</sub>                                                                                         | H                                                    | H.                                  |
| 45.             | CH <sub>3</sub>                    | CH <sub>3</sub>                   | t-C <sub>4</sub> H <sub>9</sub>                                                                         | H                                                    | H.                                  |
| 46.             | CH <sub>3</sub>                    | H                                 | n-C <sub>4</sub> H <sub>9</sub>                                                                         | H                                                    | H.                                  |
| 47.             | CH <sub>3</sub>                    | H                                 | Iso-C <sub>4</sub> H <sub>9</sub>                                                                       | H                                                    | H.                                  |
| 48.             | CH <sub>3</sub>                    | H                                 | Sec-C <sub>4</sub> H <sub>9</sub>                                                                       | H                                                    | H.                                  |
| 49.             | CH <sub>3</sub>                    | H                                 | t-C <sub>4</sub> H <sub>9</sub>                                                                         | H                                                    | H.                                  |
| 50.             | n-C <sub>4</sub> H <sub>9</sub>    | H                                 | CH <sub>3</sub>                                                                                         | H                                                    | H.                                  |
| 51.             | Iso-C <sub>4</sub> H <sub>9</sub>  | H                                 | CH <sub>3</sub>                                                                                         | H                                                    | H.                                  |
| 52.             | Sec-C <sub>4</sub> H <sub>9</sub>  | H                                 | CH <sub>3</sub>                                                                                         | H                                                    | H.                                  |
| 53.             | t-C <sub>4</sub> H <sub>9</sub>    | H                                 | CH <sub>3</sub>                                                                                         | H                                                    | H.                                  |
| 54.             | n-C <sub>5</sub> H <sub>11</sub>   | CH <sub>3</sub>                   | CH <sub>3</sub>                                                                                         | H                                                    | H.                                  |
| 55.             | Iso-C <sub>5</sub> H <sub>11</sub> | CH <sub>3</sub>                   | CH <sub>3</sub>                                                                                         | H                                                    | H.                                  |
| 56.             | Sec-C <sub>5</sub> H <sub>11</sub> | CH <sub>3</sub>                   | CH <sub>3</sub>                                                                                         | H                                                    | H.                                  |
| 57.             | t-C <sub>5</sub> H <sub>11</sub>   | CH <sub>3</sub>                   | CH <sub>3</sub>                                                                                         | H                                                    | H.                                  |
| 58.             | t-C <sub>5</sub> H <sub>11</sub>   | C <sub>2</sub> H <sub>5</sub>     | CH <sub>3</sub>                                                                                         | H                                                    | H.                                  |
| 59.             | t-C <sub>5</sub> H <sub>11</sub>   | CH <sub>3</sub>                   | Iso-C <sub>3</sub> H <sub>7</sub>                                                                       | H                                                    | H.                                  |
| 60.             | t-C <sub>5</sub> H <sub>11</sub>   | H                                 | t-C <sub>4</sub> H <sub>9</sub>                                                                         | H                                                    | H.                                  |
| 61.             | t-C <sub>5</sub> H <sub>11</sub>   | t-C <sub>4</sub> H <sub>9</sub>   | H                                                                                                       | H                                                    | H.                                  |
| 62.             | t-C <sub>5</sub> H <sub>11</sub>   | t-C <sub>4</sub> H <sub>9</sub>   | CH <sub>3</sub>                                                                                         | H                                                    | H.                                  |
| 63.             | t-C <sub>5</sub> H <sub>11</sub>   | CH <sub>3</sub>                   | t-C <sub>4</sub> H <sub>9</sub>                                                                         | H                                                    | H.                                  |
| 64.             | t-C <sub>5</sub> H <sub>11</sub>   | H                                 | n-C <sub>4</sub> H <sub>9</sub>                                                                         | H                                                    | H.                                  |
| 65.             | t-C <sub>5</sub> H <sub>11</sub>   | H                                 | Iso-C <sub>4</sub> H <sub>9</sub>                                                                       | H                                                    | H.                                  |
| 66.             | t-C <sub>5</sub> H <sub>11</sub>   | H                                 | Sec-C <sub>4</sub> H <sub>9</sub>                                                                       | H                                                    | H.                                  |
| 67.             | t-C <sub>5</sub> H <sub>11</sub>   | Iso-C <sub>3</sub> H <sub>7</sub> | t-C <sub>4</sub> H <sub>9</sub>                                                                         | H                                                    | H.                                  |
| 68.             | t-C <sub>5</sub> H <sub>11</sub>   | t-C <sub>4</sub> H <sub>9</sub>   | t-C <sub>4</sub> H <sub>9</sub>                                                                         | H                                                    | H.                                  |
| 69.             | t-C <sub>5</sub> H <sub>11</sub>   | t-C <sub>4</sub> H <sub>9</sub>   | C <sub>2</sub> H <sub>5</sub>                                                                           | H                                                    | H.                                  |
| 70.             | t-C <sub>5</sub> H <sub>11</sub>   | t-C <sub>4</sub> H <sub>9</sub>   | Iso-C <sub>3</sub> H <sub>7</sub>                                                                       | H                                                    | H.                                  |
| 71.             | t-C <sub>5</sub> H <sub>11</sub>   | t-C <sub>4</sub> H <sub>9</sub>   | t-C <sub>4</sub> H <sub>9</sub>                                                                         | H                                                    | H.                                  |
| 72.             | t-C <sub>5</sub> H <sub>11</sub>   | CH <sub>3</sub>                   | t-C <sub>4</sub> H <sub>9</sub>                                                                         | CH <sub>3</sub>                                      | H.                                  |
| 73.             | t-C <sub>5</sub> H <sub>11</sub>   | H                                 | t-C <sub>4</sub> H <sub>9</sub>                                                                         | CH <sub>3</sub>                                      | H.                                  |
| 74.             | H                                  | H                                 | t-C <sub>4</sub> H <sub>9</sub>                                                                         | CH <sub>3</sub>                                      | H.                                  |
| 75.             | t-C <sub>6</sub> H <sub>13</sub>   | H                                 | t-C <sub>4</sub> H <sub>9</sub>                                                                         | CH <sub>3</sub>                                      | H.                                  |
| 76.             | H                                  | H                                 | t-C <sub>6</sub> H <sub>13</sub>                                                                        | H                                                    | H.                                  |
| 77.             | t-C <sub>6</sub> H <sub>13</sub>   | H                                 | CH <sub>3</sub>                                                                                         | H                                                    | H.                                  |
| 78.             | H                                  | H                                 | —CH <sub>2</sub> CH=CH <sub>2</sub>                                                                     | H                                                    | H.                                  |
| 79.             | II                                 | II                                | —CH <sub>2</sub> —  | H                                                    | H.                                  |
| 80.             | OCH <sub>3</sub>                   | H                                 | H                                                                                                       | H                                                    | H.                                  |
| 81.             | H                                  | H                                 | H                                                                                                       | OCH <sub>3</sub>                                     | H.                                  |
| 82.             | H                                  | H                                 | OCH <sub>3</sub>                                                                                        | H                                                    | H.                                  |
| 83.             | OCH <sub>3</sub>                   | OCH <sub>3</sub>                  | H                                                                                                       | H                                                    | H.                                  |
| 84.             | t-C <sub>4</sub> H <sub>9</sub>    | H                                 | OCH <sub>3</sub>                                                                                        | H                                                    | H.                                  |
| 85.             | H                                  | H                                 | —O—                 | H                                                    | H.                                  |
| 86.             | COOH                               | H                                 | H                                                                                                       | H                                                    | H.                                  |
| 87.             | II                                 | H                                 | COOH                                                                                                    | H                                                    | H.                                  |
| 88.             | CH <sub>3</sub>                    | COOH                              | H                                                                                                       | H                                                    | H.                                  |
| 89.             | H                                  | COOH                              | H                                                                                                       | CH <sub>3</sub>                                      | H.                                  |
| 90.             | CH <sub>3</sub>                    | H                                 | COOH                                                                                                    | H                                                    | H.                                  |
| 91.             | t-C <sub>4</sub> H <sub>9</sub>    | t-C <sub>4</sub> H <sub>9</sub>   | COOH                                                                                                    | H                                                    | H.                                  |
| 92.             | t-C <sub>4</sub> H <sub>9</sub>    | t-C <sub>4</sub> H <sub>9</sub>   | COOH                                                                                                    | H                                                    | H.                                  |
| 93.             | H                                  | H                                 | —CH <sub>2</sub> CH <sub>2</sub> COOH                                                                   | H                                                    | H.                                  |
| 94.             | Cl                                 | Cl                                | Cl                                                                                                      | H                                                    | H.                                  |
| 95.             | H                                  | H                                 | Cl                                                                                                      | H                                                    | H.                                  |
| 96.             | H                                  | H                                 | —CH <sub>2</sub> OH                                                                                     | CH <sub>3</sub>                                      | CH <sub>3</sub> .                   |
| 97.             | t-C <sub>4</sub> H <sub>9</sub>    | t-C <sub>4</sub> H <sub>9</sub>   | —CH <sub>2</sub> OH                                                                                     | H                                                    | H.                                  |
| 98.             | —CH <sub>2</sub> OH                | —CH <sub>2</sub> OH               | —CH <sub>2</sub> OH                                                                                     | H                                                    | H.                                  |
| 99.             | t-C <sub>4</sub> H <sub>9</sub>    | t-C <sub>4</sub> H <sub>9</sub>   | —CH <sub>2</sub> OH                                                                                     | H                                                    | H.                                  |
| 100.            | t-C <sub>4</sub> H <sub>9</sub>    | H                                 | CHO                                                                                                     | H                                                    | H.                                  |
| 101.            | t-C <sub>4</sub> H <sub>9</sub>    | CH <sub>3</sub>                   | CHO                                                                                                     | H                                                    | H.                                  |
| 102.            | t-C <sub>4</sub> H <sub>9</sub>    | H                                 | —COCH <sub>3</sub>                                                                                      | H                                                    | H.                                  |
| 103.            | t-C <sub>4</sub> H <sub>9</sub>    | t-C <sub>4</sub> H <sub>9</sub>   | —COCH <sub>3</sub>                                                                                      | H                                                    | H.                                  |
| 104.            | t-C <sub>4</sub> H <sub>9</sub>    | t-C <sub>4</sub> H <sub>9</sub>   | —OOCCH <sub>3</sub>                                                                                     | H                                                    | H.                                  |
| 105.            | t-C <sub>4</sub> H <sub>9</sub>    | t-C <sub>4</sub> H <sub>9</sub>   | CH <sub>3</sub> N(CH <sub>3</sub> ) <sub>2</sub>                                                        | H                                                    | H.                                  |
| 106.            | CH <sub>3</sub>                    | H                                 | SO <sub>3</sub> H                                                                                       | H                                                    | H.                                  |
| 107.            | SO <sub>3</sub> H                  | CH <sub>3</sub>                   | CH <sub>3</sub>                                                                                         | SO <sub>3</sub> H                                    | H.                                  |
| 108.            | CH <sub>3</sub>                    | H                                 | CH <sub>3</sub>                                                                                         | SO <sub>3</sub> H                                    | H.                                  |
| 109.            | CH <sub>3</sub>                    | SO <sub>3</sub> H                 | CH <sub>3</sub>                                                                                         | CH <sub>3</sub>                                      | H.                                  |
| 110.            | CH <sub>3</sub>                    | H                                 | CH <sub>3</sub>                                                                                         | H                                                    | H.                                  |
| 111.            | H                                  | H                                 | H                                                                                                       | —NH(CH <sub>3</sub> ) <sub>2</sub> SO <sub>3</sub> H | H.                                  |
| 112.            | Br                                 | Br                                | —CH <sub>2</sub> CH <sub>2</sub> COOH                                                                   | H                                                    | H.                                  |
|                 |                                    |                                   | ↓ NH <sub>2</sub>                                                                                       |                                                      |                                     |

| Compound number | R <sub>1</sub> | R <sub>2</sub> | R <sub>3</sub> | R <sub>4</sub>                                     | R <sub>5</sub> |
|-----------------|----------------|----------------|----------------|----------------------------------------------------|----------------|
| 113             | H              | H              | H              | -N(CH <sub>3</sub> ) <sub>2</sub>                  | H              |
| 114             | H              | H              | H              | -NHC <sub>3</sub> H <sub>7</sub>                   | H              |
| 115             | H              | H              | H              | -NHCOCH <sub>3</sub>                               | H              |
| 116             | H              | H              | H              | -NHC <sub>2</sub> H <sub>4</sub> COCH <sub>3</sub> | H              |



Pat. No. 3790383



| Compound number | R <sub>1</sub>                  | R <sub>2</sub> | R <sub>3</sub>  | R <sub>4</sub>                  | R <sub>5</sub> |
|-----------------|---------------------------------|----------------|-----------------|---------------------------------|----------------|
| 130             | t-C <sub>4</sub> H <sub>9</sub> | H              |                 | t-C <sub>4</sub> H <sub>9</sub> | H              |
| 131             | t-C <sub>4</sub> H <sub>9</sub> |                | CH <sub>3</sub> | H                               | H              |
| 132             | t-C <sub>4</sub> H <sub>9</sub> | H              |                 | t-C <sub>4</sub> H <sub>9</sub> | H              |
| 133             | t-C <sub>4</sub> H <sub>9</sub> |                | CH <sub>3</sub> | H                               | H              |

These compounds which are all known are described in "The Inhibition of Fat Oxidation Processes" written by N.M. Emanuel and Y.N. Lyaskovskaya (Pergamon Press Ltd., 1967) and "Atmospheric Oxidation and Antioxidation" written by G. Scott (Elsevier Publ. Co., 1965). They are commonly available.

Practical uses for the compounds used in the present invention were heretofore unknown. Especially, it has not been known at all to improve the preservability of a developer by adding the compounds to any developer, not to mention a developer for photographic plate for printing.

As the result of examinations regarding many kinds of compounds, the present inventors have found that the preservability of the developer is improved by using compounds of the above-described general formula. The reason why the preservability is improved by addition of these compounds to the developer of the photographic plate for printing is unknown.

The preservability of the developer, however, is greatly improved as compared to the use of known preservatives such as sodium sulfite, ascorbic acid, etc., and the resulting photographic images have excellent quality with low fringe and excellent dots. Moreover, delay in the progress of the development which is observed with prior art developers is not observed when using the compounds of the present invention.

Though any compound of the present invention represented by the above-mentioned formula is effective for improving the preservability of infectious developers, those which are substituted by at least one alkyl group are preferred and those having an alkyl group with many carbon atoms are most preferred and specific carbon ranges of more preferred groups are more than 2. In this case, the solubility of the compound is important. For the purpose, water-soluble groups such as sulfon, carboxyl or hydroxyalkyl groups may be bonded to the nuclei with the substituted hydrocarbon. The most preferred carbon ranges are 3 to 5.

Further, compounds in which the ortho positions of the benzene ring is substituted by one or preferably two alkyl groups are especially effective. Among these compounds, sterically hindered phenols such as those having an isopropyl group, a t-butyl group or a t-amyl group are especially preferred. It is also especially ef-

fective to introduce a sulfo group, a carboxyl group or a hydroxyalkyl group in addition to the alkyl groups in order to increase the water-solubility of these compounds.

The water-soluble cations are an alkali metal such as sodium or potassium, and ammonium group.

The developer for photographic plates for printing to which the compounds of the present invention are added is the common infectious developer which contains hydroquinone as the developing agent. The developer may also contain water-soluble acids, alkalies and salts such as sodium carbonate, sodium hydroxide, acetic acid and boric acid as an alkali agent or a pH buffer agent, aldehyde-alkali hydrogen sulfite addition products, ketone-alkali hydrogen sulfite addition products, sulfites or two or more thereof as an antioxidant, and alkali halides as a development controlling agent in addition to the hydroquinone. The developer may contain, if desired, organic antifogging agents such as benzotriazole and 1-phenyl-5-mercapto-tetrazole, polyalkylene oxides, amine compounds or organic solvents such as triethylene glycol, dimethylformamide, methyl alcohol and cellosolve in the amount of 1 - 300 ml per liter of the developer.

The primary characteristic of prior art infectious developer is to have a low free sulfite ion concentration as shown above. Therefore, a sulfite ion buffer such as a formaldehyde-sodium hydrogen sulfite addition product is used. In general, the free sulfite ion concentration is controlled by additionally adding sulfite such as alkali sulfite, for example, sodium sulfite or potassium sulfite, because sulfite is added to be in the presence of sulfite ion to the sulfite ion buffer in the amount of less than 5 g per liter of the developer. Of course, sulfite is not necessarily added to the developer and, if it is added, the amount thereof is 5 g or less, especially 1 to 3 g, per one liter of the developer. Sulfite ion buffer is an aldehyde-alkali hydrogen sulfite addition product such as formaldehyde-sodium hydrogen sulfite addition product, or a ketone-alkali hydrogen sulfite such as acetone-sodium hydrogen sulfite addition product. Other examples of addition products are described in U.S. Pat. No. 3,573,914. Usually up to about 3 g of sulfite is added by which the preservability of the developer is somewhat improved, though the quality of half-tone dots somewhat deteriorates. However, as shown

above, such a degree of preservability is not satisfactory. According to the present invention, the preservability is remarkably improved by adding the above-mentioned compounds to the infectious developer containing no alkali sulfite other than a sulfite ion buffer such as formaldehyde-sodium sulfite addition product, and the preservability can be remarkably improved by adding to the infectious developer less than 5 g (per liter of the developer) of an alkali sulfite in addition to the sulfite ion buffer. Sulfite may be added to the developer with the compound of the invention, whereby the developer shows stronger preservability than that containing only sulfite.

Essential components of the infectious developer are hydroquinone, an addition product and the compound of the invention.

A range of hydroquinone is 5 to 50 g, preferably 10 to 30 g, per one liter of developer.

A range of additional product is 10 to 100 g, preferably 30 to 70 g, per one liter of developer.

In the above essential components, alkali should be added, but the amount thereof may be such amount that pH of the developer is alkali property, especially pH 8 or more, and more preferably pH 9 - pH 11.

In the present invention, more than one compound of the present invention can be used at one time. Though the amount of the compounds in the present invention depends upon a composition of the developer and the kind of the compound, about 2 mg to about 20 g of the compound per liter of the developer is generally used. The most preferred amount is 10 mg to about 5 g or so.

In general, the compounds in the present invention are added at the preparation of the developer. In the case that the developer is prepared as a liquid or powder composition and mixed, diluted or dissolved at the time of use, it is effective at that time to previously add the compounds of the present invention to the composition. In the case of using a liquid composition, it is particularly effective to add the compounds to such a liquid composition because the preservability of the liquid composition is remarkably increased by the addition of the compounds. Common liquid compositions consist of two liquids, that is, one part containing the developing agent, a second part containing an alkali. Although the compound of the present invention may be added to either part, it is more preferred to add to the part containing the developing agent, by which the preservability of the liquid developer can be further improved and the stability of the developer after preparation of the infectious developer by dilution can be remarkably improved. As another method, it is possible to improve the preservability of the developer by adding the compounds of the present invention during or after development of the photographic plate for printing.

As emulsions used to form photographic plates for printing, common silver halide photographic emulsions are used, in which silver chloride, silver bromide, silver chlorobromide, silver bromoiodide and silver chloro-

bromoiodide can be used. Particularly, silver chlorobromide is suitably used. These silver halides are dispersed in gelatin or a medium comprising gelatin and a synthetic high molecular substance to form an emulsion. The emulsion may be chemically sensitized by compounds containing unstable sulfur such as sodium thiosulfate and allyl thiourea, gold compounds such as complex salt of monovalent gold and thiocyanate, or combinations thereof. The emulsions may be optically sensitized by adding an optical sensitizing agent such as cyanine dyes, merocyanine dyes, etc. Furthermore, the emulsions may be hardened with a hardening agent such as formaldehyde or mucochloric acid, and may contain surface active agents such as saponin so as to make application easy. These additives are added for their well known prior art functions in conventional amounts.

The following examples of the present invention are presented to illustrate the excellent effects of the present invention.

#### EXAMPLE 1

After photographing an exposure wedge used for sensitometry through a 150-line magenta contact screen using an available lithofilm, the film was developed at 20° C by 4 kinds of developers having the following compositions. The litho film can be prepared by coating on a support a gelatino silver chlorobromoiodide emulsion (AgCl 75 mol percent, AgBr 0.2 mol percent) sensitized with gold and sulfur and then spectrally sensitized with 3-carboxymethyl-5-[2-(3-ethylthiazolinidene)-ethylidene] rhodamine, said emulsion containing polyoxyethylene nonylphenyl ether having ethylene oxide group number of 50, mucochloric acid and polybutylmethacrylate.

#### Developer A

|                                                       |      |
|-------------------------------------------------------|------|
| Sodium carbonate (monohydrate)                        | 50 g |
| Formaldehyde-sodium hydrogen sulfite addition product | 45 g |
| Potassium bromide                                     | 2 g  |
| Hydroquinone                                          | 18 g |
| Sodium sulfite                                        | 2 g  |
| Water to make 1 liter                                 |      |

#### Developer B

Same as Developer A with 0.05 g of Compound 61 of the present invention added.

#### Developer C

Same as Developer A with 2 g of sodium sulfite added.

#### Developer D

Same as Developer A with 1 g of L-ascorbic acid added.

The photographic properties obtained using each developer are shown in Table 1.

TABLE I

| Developer | Additives       | Amount (g/l) | Time of development (minute) | Quality of half-tone dot | Fresh liquid | Sensitivity<br>Elapsed liquid |
|-----------|-----------------|--------------|------------------------------|--------------------------|--------------|-------------------------------|
| A         | —               | —            | 2%                           | a                        | 100          | 34                            |
| B         | Compound 61     | 0.05         | 2%                           | a                        | 100          | 95                            |
| C         | Sodium sulfite  | 3.0          | 3                            | c                        | 100          | 52                            |
| D         | L-Ascorbic acid | 1.0          | 3                            | a                        | 100          | 50                            |

The time of development was that necessary to reach the sensitivity obtained by developing for 2 3/4 minutes with Developer A (this sensitivity is regarded as 100). The quality of the half-tone dots is denoted by 3 ranks a, b and c, that is, a means excellent, b means fairly good and c means worse. The term elapsed liquid means the developer has been subjected to deterioration by contacting 500 ml of the developer in a 20 cm X 25 cm development vat with the air for 5 hours.

As is clear from Table 1, the sensitivity of Developer A (control) deteriorates largely with lapse of time. The sensitivity of comparison prior art Developer C in which 20 g of sodium sulfite is added lowers considerably with lapse of time, though deterioration is less than that of Developer A. Further, the efficiency of half-tone dot formation in the fresh liquid is worse than for Developer A. Deterioration of the sensitivity of Developer D in which 1.0 g of L-ascorbic acid is added is nearly equal to that of Developer C, not yet satisfactory.

In Developer B, containing 0.05 g of Compound 61 of the present invention, deterioration of sensitivity with lapse of time is the lowest and the deterioration of the quality of the half-tone dots in the fresh liquid is not observed to any significant extent.

#### EXAMPLE 2

After photographing an exposure wedge for sensitometry through a 150-line contact screen using an available lithofilm, the film was developed at 20° C using developers prepared from two kinds of components having the following compositions.

#### Developer E

| Solution I                                            |        |
|-------------------------------------------------------|--------|
| Distilled water                                       | 60 ml  |
| Triethylene glycol                                    | 30 ml  |
| Formaldehyde-sodium hydrogen sulfite addition product | 45 g   |
| Hydroquinone                                          | 16 g   |
| Distilled water to make                               | 125 ml |

  

| Solution II                    |        |
|--------------------------------|--------|
| Distilled water                | 100 ml |
| Sodium carbonate (monohydrate) | 30 g   |
| Sodium hydroxide               | 5 g    |
| Boric acid                     | 3 g    |
| Sodium bromide                 | 2 g    |
| Distilled water to make        | 125 ml |

At use, Solution I was added to 750 ml of water and Solution II was added thereto to provide 1 liter of the final solution to be used.

#### DEVELOPER F:

That obtained by adding 0.2 g of Compound 29 of the present invention to Solution I of Developer E prior to forming the final developer.

10 The resulting photographic properties are shown in Table 2.

Deterioration in the sensitivity of the developer containing Compound 29 is less than that of the developer not containing the compound.

#### EXAMPLE 3

20 After photographing an exposure wedge for sensitometry through a 150-line contact screen using an available lithofilm, the film was developed at 20° C with developers having the following compositions.

#### Developer G

|    |                                                       |      |
|----|-------------------------------------------------------|------|
| 30 | Sodium carbonate (monohydrate)                        | 40 g |
|    | Formaldehyde-sodium hydrogen sulfite addition product | 60 g |
|    | Potassium bromide                                     | 2 g  |
|    | Boric acid                                            | 3 g  |
|    | Hydroquinone                                          | 18 g |
| 35 | Sodium sulfite                                        | 2 g  |
|    | Water to make 1 liter                                 |      |

#### DEVELOPERS H, I, J, K, L, M AND N:

Those were prepared by adding Compounds 71, 74, 82, 86, 93, 96 and 98, respectively, to Developer G. The results of development are shown in Table 3.

TABLE 2

| Developer | Additive    | Amount (g/l) | Time of development (minute) | Quality of half-tone dot | Sensitivity  |                |
|-----------|-------------|--------------|------------------------------|--------------------------|--------------|----------------|
|           |             |              |                              |                          | Fresh liquid | Elapsed liquid |
| E         | —           | —            | 2 1/2                        | a                        | 100          | 31             |
| F         | Compound 29 | 0.2          | 2 1/2                        | a                        | 100          | 90             |

TABLE 3

| Developer | Additive     | Amount (g/l) | Time of development (minute) | Quality of half-tone dot | Sensitivity  |                |
|-----------|--------------|--------------|------------------------------|--------------------------|--------------|----------------|
|           |              |              |                              |                          | Fresh liquid | Elapsed liquid |
| G         | —            | —            | 2 1/2                        | a                        | 100          | 35             |
| H         | Compound 71  | 0.02         | 2 1/2                        | a                        | 100          | 95             |
| I         | Compound 74  | 1.10         | 2 1/2                        | a                        | 100          | 90             |
| J         | Compound 82  | 1.20         | 2 1/2                        | a                        | 100          | 75             |
| K         | Compound 86  | 2.00         | 2 1/2                        | a                        | 100          | 74             |
| L         | Compound 93  | 2.00         | 2 1/2                        | a                        | 100          | 73             |
| M         | Compound 96  | 2.00         | 2 1/2                        | a                        | 100          | 80             |
| N         | Compound 108 | 1.50         | 2 1/2                        | a                        | 100          | 75             |

In the developers containing the compounds of the present invention the quality of the half-tone dots did not lower and deteriorate in sensitivity with lapse of time being low, meaning excellent preservability.

## EXAMPLE 4

After photographing an exposure wedge for sensitometry through a 150-line contact screen with an available lithofilm, the film was developed at 20°C with developers having the following compositions.

## Developer O

| Solution I                                            |        |  |
|-------------------------------------------------------|--------|--|
| Distilled water                                       | 50 ml  |  |
| Dimethylformamide                                     | 30 ml  |  |
| Formaldehyde-sodium hydrogen sulfite addition product | 45 g   |  |
| Potassium sulfite                                     | 2 g    |  |
| Hydroquinone                                          | 16 g   |  |
| Distilled water to make                               | 125 ml |  |
| <br>Solution II                                       |        |  |
| Distilled water                                       | 100 ml |  |
| Potassium carbonate                                   | 40 g   |  |
| Potassium hydroxide                                   | 4 g    |  |
| Glacial acetic acid                                   | 2 ml   |  |
| Potassium bromide                                     | 2 g    |  |
| Distilled water to make                               | 125 ml |  |

At use, Solution I is added to 750 ml of water and Solution II is added to provide 1 liter of a solution to be used.

## DEVELOPERS P, Q, R, S AND T

These were prepared by adding Compounds 117, 121, 131, 132 and 133, respectively, in an amount of 0.03 g/l to Solution I of Developer O prior to combination with water and solution. The results of development are shown in Table 4.

amount of hydroquinone does not lower as much, and the developer endures for long periods of preservation.

## EXAMPLE 6

25 l. of Developer E in Example 2 was supplied to two automatic developing devices for plate making. 200 sheets of half-cut lithofilm were treated while adding a supplementary solution having the following composition in an amount of 70 ml per sheet of half-cut lithofilm.

## Supplementary solution

| Solution I                                            |        |  |  |
|-------------------------------------------------------|--------|--|--|
| Distilled water                                       | 45 ml  |  |  |
| Triethyleneglycol                                     | 45 ml  |  |  |
| Formaldehyde sodium hydrogen sulfite addition product | 45 g   |  |  |
| Hydroquinone                                          | 20 g   |  |  |
| Distilled water to make                               | 125 ml |  |  |
| <br>Solution II                                       |        |  |  |
| Distilled water                                       | 100 ml |  |  |
| Sodium carbonate                                      | 30 g   |  |  |
| Sodium hydroxide                                      | 5 g    |  |  |
| Boric acid                                            | 1 g    |  |  |
| Distilled water to make                               | 125 ml |  |  |

At use, Solution I was added to 750 ml of water and Solution II was then added thereto to provide 1 liter of the solution to be used.

After developing the lithofilm, one of the automatic developing devices was left as it stands, and 75 ml of a 1 percent methanol solution of Compound 62 of the present invention was added to the other automatic developing apparatus. After leaving both automatic developing devices for 64 hours, the lithofilms were then

TABLE 4

| Developer | Additive     | Amount (g/l) | Time of development (minute) | Quality of half-tone dot | Fresh liquid | Sensitivity<br>Elapsed liquid |
|-----------|--------------|--------------|------------------------------|--------------------------|--------------|-------------------------------|
| O         |              |              | 2%                           | a                        | 100          | 34                            |
| P         | Compound 117 | 0.03         | 2%                           | a                        | 100          | 73                            |
| Q         | Compound 121 | 0.03         | 2%                           | a                        | 100          | 74                            |
| R         | Compound 131 | 0.03         | 2%                           | a                        | 100          | 85                            |
| S         | Compound 132 | 0.03         | 2%                           | a                        | 100          | 97                            |
| T         | Compound 133 | 0.03         | 2%                           | a                        | 100          | 92                            |

In the developers containing the compounds of the present invention the quality of the half-tone dots was not lowered and deterioration in the sensitivity with lapse of time was low, meaning excellent preservability.

## EXAMPLE 5

Each of Solutions I of Developer E and F in Example 2 were put into a vat and exposed to air. After standing at 50°C for 20 days, a reduced amount of hydroquinone as the developing agent was determined. The results are shown in Table 5.

TABLE 5

| Developer   | Remaining amount of hydroquinone (%) |
|-------------|--------------------------------------|
| Developer E | 90                                   |
| Developer F | 99                                   |

It is clear from Table 5 that in concentrated Solution I containing Compound 29 of the present invention, the

developed. In the developing apparatus to which the compound of the present invention was added, deterioration of the sensitivity was not observed at all, but in the developing apparatus to which the compound of the present invention was not added, notable deterioration of the sensitivity was observed. Same results as in the former examples could be obtained.

While the invention has been particularly shown and described with reference to preferred embodiments thereof, it will be understood by those skilled in the art that various changes in form and details may be made therein without departing from the spirit and scope of the invention.

What is claimed is:

1. An infectious developer for photographic plates for use in printing which comprises:
  1. hydroquinone as the sole developing agent,
  2. a free sulfite in a concentration of less than 5

- grams per liter, and  
 3. at least one phenol compound represented by the following formula:



wherein R<sub>1</sub>, R<sub>2</sub>, R<sub>3</sub>, R<sub>4</sub> and R<sub>5</sub>, which need not be identical, represent a member selected from the group consisting of a hydrogen atom, a lower alkyl group, a lower alkoxy group, a COOM group, an SO<sub>3</sub>M group wherein M represents a member selected from the group consisting of a hydrogen atom, a water-soluble cation, a lower alkyl group, a halogen atom, an S-R<sub>6</sub> group wherein R<sub>6</sub> is identical to the phenol residue to which the S atom is affixed and a COR<sub>7</sub> group wherein R<sub>7</sub> represents a member selected from the group consisting of a hydrogen atom and a lower alkyl group.

2. The developer of claim 1 wherein said developer further contains a member selected from the group consisting of an aldehyde-alkali hydrogen sulfite addition product and a ketone-alkali hydrogen sulfite addition product.

3. The developer of claim 1 wherein said developer has a pH of from 9 to 11.

4. The developer of claim 1 wherein said phenol compound has at least one alkyl group having more than 2 carbon atoms.

5. The developer of claim 4 wherein said alkyl group has a carbon range of from 3 to 5 carbon atoms.

6. The developer of claim 5 wherein said alkyl group is a member selected from the group consisting of an isopropyl group, a t-butyl group and a t-amyl group.

7. The developer of claim 1 wherein said phenol

20

25

30

35

40

45

50

55

60

65

compound has a water-soluble group attached thereto, selected from the group consisting of a sulfone group, a carboxy group and a hydroxyalkyl group.

8. The developer of claim 1 wherein at least one of R<sub>1</sub> and R<sub>2</sub> in said phenol compound is a lower alkyl group.

9. A method for developing a photographic printing plate which comprises:

10. 1. exposing said plate so as to obtain a latent image and

2. developing said exposed plate with an infectious developer comprising:

a. hydroquinone as the sole developing agent,

b. a free sulfite in a concentration of less than 5 grams per liter, and

c. at least one phenol compound represented by the following formula:



wherein R<sub>1</sub>, R<sub>2</sub>, R<sub>3</sub>, R<sub>4</sub> and R<sub>5</sub>, which need not be identical, represent a member selected from the group consisting of a hydrogen atom, a lower alkyl group, a lower alkoxy group, a COOM group, an SO<sub>3</sub>M group wherein M represents a member selected from the group consisting of a hydrogen atom, a water-soluble cation, a lower alkyl group, a halogen atom, an S-R<sub>6</sub> group wherein R<sub>6</sub> is identical to the phenol residue to which the S atom is affixed and a COR<sub>7</sub> group wherein R<sub>7</sub> represents a member selected from the group consisting of a hydrogen atom and a lower alkyl group.

\* \* \* \* \*